



be soluble, particularly in the case of the oligomers having two strongly polar groups.

Examples of the salts of interest are sodium, potassium, calcium, zinc, magnesium, barium, and the lower alkyl and alkanol substituted amines, such as, ethanol amine. One skilled in the art may readily determine which of the oligomers of the invention and which of their salts are water soluble.

A particularly preferred class of oligomers which are useful as emulsifiers have the formula:



where R is a primary or secondary alkyl having from 6 to 12 carbon atoms, preferably a normal alkyl group having from 7 to 11 carbon atoms, and, most desirably, 8 or 10 carbon atoms; R<sub>1</sub> is either hydrogen or methyl; a+b, the degree of polymerization, is broadly from 4 to 50, preferably from 12 to 30, and

$$\frac{a}{a+b}$$

is 0 to 0.6, most preferably 0.2 to 0.55. For use as an emulsifier this class of oligomers is converted to the water

soluble ammonium, lower alkyl and alkanol substituted ammonium, or alkali metal salts.

Another preferred class of oligomers has the formula:



where R is a primary or secondary alkyl, preferably a normal alkyl group having from 6 to 20 carbon atoms, and, preferably, from 7 to 12 carbon atoms; R<sub>1</sub> is either hydrogen, methyl or —CH<sub>2</sub>COOH; R<sub>2</sub> is hydrogen or methyl; a+b, the degree of polymerization, is broadly from 6 to 50, preferably from 12 to 30 and

$$\frac{a}{a+b}$$

is .075 to .40 most preferably 0.075 to .30. When a mono-function acid is present the upper portion of the ranges are preferred while for difunctional acid the lower portions are preferred.

Since this class is water soluble it may be used in its acid form or converted into its water soluble salts as described above.

Examples of the compounds of the instant invention are:

|               | $\frac{a}{a+b}$ | $\frac{a}{a+b}$ |
|---------------|-----------------|-----------------|
| (1)-----<br>  | 16              | 0.5             |
| (2)-----<br>  | 20              | 0.4             |
| (3)-----<br>  | 10              | 0.0             |
| (4)-----<br>  | 10              | 0.0             |
| (5)-----<br>  | 20              | 0.25            |
| (6)-----<br>  | 20              | 0.25            |
| (7)-----<br>  | 20              | 0.1             |
| (8)-----<br>  | 20              | 0.2             |
| (9)-----<br>  | 20              | 0.2             |
| (10)-----<br> | 20              | 0.1             |
| (11)-----<br> | 20              | 0.2             |
| (12)-----<br> | 15              | 0.0             |
| (13)-----<br> | 15              | 0.0             |

TABLE—Continued

|                                                                                                  | <i>a</i> | <i>a</i>   |                 |
|--------------------------------------------------------------------------------------------------|----------|------------|-----------------|
|                                                                                                  |          | <i>a+b</i> | $\frac{a}{a+b}$ |
| (14)-----<br>   |          | 15         | 0.0             |
| (15)-----<br>   |          | 15         | 0.0             |
| (16)-----<br>   | 40       | 0.05       |                 |
| (17)-----<br>   | 20       | 0.2        |                 |
| (18)-----<br>   | 20       | 0.2        |                 |
| (19)-----<br>   | 20       | 0.1        |                 |
| (20)-----<br>   | 40       | 0.15       |                 |
| (21)-----<br>  | 40       | 0.2        |                 |
| (22)-----<br> | 40       | 0.2        |                 |
| (23)-----<br> | 40       | 0.15       |                 |
| (24)-----<br> | 15       | 0.2        |                 |
| (25)-----<br> | 40       | 0.15       |                 |

In preparing the compounds of the instant invention an alkyl mercaptan is reacted with one or more alpha, beta double-bonded monomers. As can be seen from the discussion above one monomer unit must contain a strongly polar group. Examples of these monomers are: acrylic acid, methacrylic acid, alpha-ethylacrylic acid, beta-methyl-acrylic acid, alpha-beta dimethylacrylic acid, hexanoic acid, itaconic acid, maleic acid, fumaric acid, acrylamide, methacrylamide, vinyl ethyl ether, vinyl methyl ether, vinyl pyrrolidone, and allyl alcohol.

Where a second monomer is used it may also be selected from the aforesaid group of strongly polar compounds or be a less polar material such as acrylonitrile, or methylacrylonitrile, ethylacrylonitrile, methyl acrylate, ethyl acrylate, methyl methacrylate, hydroxyethyl acrylate, hydroxypropyl acrylate, hydroxyethyl methacrylate, hydroxypropyl methacrylate, vinyl acetate, vinyl propionate, N-isopropyl-acrylamide, N-ethyl acrylamide, N-methyl acrylamide, N-methylolacrylamide, glycidyl acrylate, glycidyl methacrylate.

60

The reaction is performed in an essentially water-free reaction medium, preferably, in a lower alcohol having a boiling point of less than 100° C., e.g., methanol, ethanol and propanol. Other solvents which dissolve the reactants and the catalyst may also be advantageously used.

Generally, the oligomerization temperature is maintained at 20–60° C. Temperature of up to 100° C. may be used. Optimum temperature may readily be determined for each polymerization and depend on the reaction and relative reactivity of the monomers. In order to facilitate the free radical propagation necessary for an effective catalytic reaction an oxygen-free atmosphere is desirable. This may be obtained by bubbling an inert gas such as nitrogen through the reaction system.

The catalyst employed must be a free radical initiator, such as the peroxides and persulfates. These materials are well known in the art. As required, activators may be added as, for example, N,N'-dimethylaniline. Particularly outstanding results are obtained with organic peroxides and hydroperoxides, hydrogen peroxide, diazo such

65

70

75

as diazo bis(isobutyronitrile) and water soluble persulfates. Specific examples include ammonium persulfate, the alkali metal and alkaline earth metal persulfates and the alkyl peroxides such as lauroyl peroxide, cyclohexyl peroxide and t-butyl peroxide. Catalytic amounts of initiator are used, i.e., between 0.1 to 6.0 grams per total mole depending on the particular initiator and the monomers system. For example from 0.1 to 0.5 grams of the ammonium persulfate catalyst are employed per gram mole of monomer (calculated as total moles monomers). If the catalyst is lauroyl peroxide the range is .5 to 6.0 g. While lesser amounts can be used, it will decrease the conversion. Greater amounts give no significant advantage.

A convenient method for carrying out the reaction is to dissolve the alkyl mercaptan initially and the monomer or monomers, as the case may be, in the alcoholic solvent. Thereafter, the catalyst, also dissolved in the solvent, is added slowly. Upon completion of the reaction, the reaction product, if it is homogeneous, may be treated with an aqueous base, as for example an alkali metal hydroxide, such as potassium hydroxide, to neutralize the acid present to a pH of from about 6.5 to 8.5. By vacuum stripping the solvent may be separated leaving a water solution of the salt, e.g., the potassium salt, of the oligomers of the instant invention. However, if the reaction product is heterogeneous, as for example some oligomers precipitate out of the alcohol solvent as they are formed, the product may be isolated by filtration, washing and drying. These products may dissolve in water without the use of an alkali metal hydroxide.

#### EXAMPLE I

Low molecular weight polymers (i.e., oligomers) of the invention having the general formula  $n$ -alkyl-S-[acrylonitrile]<sub>a</sub>-[acrylic acid]<sub>b</sub>-H are prepared in metha-

Following the procedure outlined above the reaction is initiated at the reaction temperature by introducing a solution of the initiator at a rate of 38 ml./hr. A total of 0.232 gms. ammonium persulfate per mole of monomer (calcd. as moles of acrylonitrile and acrylic acid only) are added. This equals a total of 2.5 g. of ammonium persulfate.

The transparent greenish-yellow reaction mix is determined to be 65.0% solids, as compared to a theoretical solids content of 65.3%, showing an essentially 100% conversion. The viscosity of the mix is about 1000 cp. After evaporation to dryness at 100° C./2 mm. for 30 minutes, a white, friable powder, soluble in methanol, acetone, methyl ethyl ketone and cyclohexanone, remains. By vapor phase osmometry the number average molecular weight is found to be about 1100 as compared to a calculated value of 1146. Analysis shows the reaction product contains 50% acrylic acid, 36.5% acrylonitrile and 13.5% n-octyl mercaptan and is essentially pure. This material upon conversion to the potassium salt is a useful surface active agent.

#### Run 2—n-octyl-S-[acrylonitrile]<sub>3</sub>-[acrylic acid]<sub>3</sub>-H

Following the procedure described in Run 1, 115 g. (1.6 moles) acrylic acid, 84.8 g. (1.6 moles) acrylonitrile, 77.87 g. (0.533 moles) n-octyl mercaptan and 16 g. methanol are added to the reaction flask. 147 ml. of an ammonium persulfate solution (0.66 gms.  $(NH_4)_2S_2O_8$ /100 ml. methanol) are added during the 5½ hours of the reaction. This is equivalent to 0.303 g./mole of monomer. The solids obtained are 63.3% indicating a conversion of 93.5%.

Additional runs for preparing R-S-(acrylonitrile)<sub>a</sub>-(acrylic acid)<sub>b</sub>-H, all using the general procedure described above, are shown in the following Table 1;

TABLE 1  
[Preparation of R-S-(acrylonitrile)<sub>a</sub>-(acrylic acid)<sub>b</sub>-H oligomers]

| Run No. | R         | $a+b$ | $a/a+b$ | Materials loaded, g. |                    |      | 0.66 g. $(NH_4)_2S_2O_8$<br>per 100 ml. methanol | Reaction    |                     | Percent<br>conversion |      |
|---------|-----------|-------|---------|----------------------|--------------------|------|--------------------------------------------------|-------------|---------------------|-----------------------|------|
|         |           |       |         | Acrylic<br>acid      | Acrylo-<br>nitrile | RSH  |                                                  | Ml.<br>used | G./mole<br>monomers |                       |      |
| 3       | N-Octyl   | 10    | 0.5     | 144                  | 106                | 58.4 | 20                                               | 147         | 0.243               | 35                    | 53/4 |
| 4       | do        | 14    | 0.4     | 172.8                | 84.8               | 41.8 | 14                                               | 157         | 0.086               | 35                    | 71/4 |
| 5       | do        | 14    | 0.5     | 144                  | 106                | 41.8 | 35                                               | 124.5       | 0.205               | 35                    | 52/3 |
| 6       | do        | 20    | 0.5     | 129.6                | 95.4               | 26.3 | 36                                               | 71          | 0.126               | 35                    | 82/3 |
| 7       | n-Dodecyl | 14    | 0.5     | 144                  | 106                | 57.8 | 20                                               | 105         | 0.174               | 30                    | 99.7 |
| 8       | do        | 20    | 0.4     | 129.6                | 63.6               | 30.3 | 25                                               | 44          | 0.097               | 35                    | 53/4 |
| 9       | do        | 20    | 0.5     | 120.6                | 95.4               | 36.4 | 36                                               | 78          | 0.138               | 35                    | 98.2 |
| 10      | n-Decyl   | 16    | 0.5     | 144                  | 106                | 43.5 | 41                                               | 146         | 0.240               | 35                    | 52/3 |
| 11      | do        | 30    | 0.5     | 216                  | 159                | 34.8 | 61.5                                             | 200         | 0.220               | 35                    | 71/4 |
| 12      | do        | 16    | 0.25    | 216                  | 53                 | 43.5 | 133                                              | 132         | 0.218               | 35                    | 51/2 |

<sup>1</sup> The initiator solution used in this run was 0.22 g.  $(NH_4)_2S_2O_8$ /100 ml. methanol.

<sup>2</sup> The initiator solution used in this run was 0.64 g.  $(NH_4)_2S_2O_8$ /100 ml. methanol.

not using ammonium persulfate as the initiator. The general procedure employed is to add the acrylic acid, acrylonitrile, n-alkyl mercaptan and methanol solvent to a reaction flask which is immersed in a water bath and equipped with an additional funnel, a thermometer, an agitator, a water-cooled condenser and a nitrogen inlet. The solution is agitated, the nitrogen flow commences, and the contents of the flask is heated. When reaction temperature, in this example 35° C., is reached, a solution of the initiator in the methanol is introduced at a controlled rate into the flask via the addition funnel. Because the reaction gives off heat, it is necessary to control the water bath in order to maintain a constant oligomerization temperature.

#### Run 1—Preparation of n-octyl-S-[acrylonitrile]<sub>8</sub>-[acrylic acid]<sub>8</sub>-H

The following materials are added to the reaction flask:

388.8 g. (5.4 moles) acrylic acid  
286.2 g. (5.4 moles) acrylonitrile  
98.6 g. (0.675 moles) n-octyl mercaptan  
110.7 g. methanol

Using the same reaction flask as described in Example I, additional low molecular weight compounds are prepared. In these runs the solvent is isopropanol and the initiator lauroyl peroxide.

#### Run 1—n-Octyl-S-[acrylonitrile]<sub>8</sub>-[acrylic acid]<sub>12</sub>-H

The following materials are added to the reaction flask:

907.2 gm. (12.6 moles) acrylic acid  
445.2 gm. (8.4 moles) acrylonitrile  
153.2 gm. (1.05 moles) n-octyl mercaptan  
10.5 gm. (0.5 gm./mole of monomers) lauroyl peroxide  
420 gm. isopropanol

The flask is heated to 50° C. by means of the water bath.

After 3½ hours it is noted that the reaction mix becomes very viscous. At this time an additional 591 grams of isopropanol are added. After 4.8 hours 204.1 grams (2.835 mols) of acrylic acid and 136.1 grams isopropanol are added. Additional initiator, namely, 5.25 grams (0.25

grams per mole of monomer) of lauroyl peroxide are added after 5½ hours. At the end of 9 hours the bath is cooled from the reaction temperature to 30° C. It remains at this temperature until the end of the run. After 24 hours the conversion is 94.8%.

The reaction product is a transparent yellowish liquid which contains 56.9% solids and has a viscosity of 16,500 centipoises. After drying the reaction product for 30 minutes at 100° C. at 2 mm. pressure, a solid is obtained which was 62.1% acrylic acid, 9.7% n-octylmercaptan and 25.3% acrylonitrile (a total of 97.1%). The intrinsic viscosity in isopropanol of this powder is 0.056. This reaction product can be used as an emulsifier by stripping off the solvent from the aqueous neutralized reaction mixture as described for run 1 in Example I. KOH is used for the neutralization.

Run 2—n-Octyl-S-[acrylic acid]<sub>10</sub>-H

In a laboratory reactor are placed 72 g. acrylic acid (1 mole), 14.6 g. (0.1 mole) n-octyl mercaptan, 1.5 g. lauroyl peroxide (1.5 g./mole of monomer), and 350 ml. isopropanol. This is heated by a 40° C. water bath. When the temperature of flask reaches 40° C., 7 drops of N,N-dimethyl aniline (DMA) are added. After 25 minutes, the reaction starts and the temperature reaches 48.5° C. at 45 min. then falls to 40.9° C. at 3 hours. 15 drops of DMA are then added, but no exotherm results. The reaction product is diluted with water and stripped free of isopropanol without neutralization. It is soluble in water in its acidic form.

Run 3—n-Octyl-S-[acrylic acid]<sub>20</sub>-H

In a laboratory reactor are placed 46.3 g. acrylic acid (0.6429 moles), 4.7 g. n-octyl mercaptan (0.032 moles), 1.1 g. lauroyl peroxide, (1.7 g./mole of monomers), and 353.7 g. isopropanol. This is heated by means of a water bath to 39.9° C. and 11 drops of DMA are then added. The temperature of the reaction rises to 40.8° C. in thirty minutes, is held at this temperature for 45 minutes and falls to 40.2° C. during the ensuing 75 minutes. At that time, the addition of 1 g. lauroyl peroxide and 10 drops DMA produces a temperature rise to 40.4° C. The reaction is continued for 3 hours.

The reaction product is diluted with water and stripped without neutralization to remove the isopropanol. It is soluble throughout this process. A 1% solution has the following surface tensions at the indicated K<sup>+</sup>pH: 33 d./cm. at pH 3.2; 39 d./cm. at pH 9.5.

Run 4—n-Octyl-S-[acrylonitrile]<sub>10</sub>-[acrylic acid]<sub>10</sub>-H

In a bottle reactor are placed 36 g. acrylic acid (0.5 moles), 26.5 g. acrylonitrile (0.5 moles), 7.3 g. n-octyl mercaptan (0.05 moles), 6 g. lauroyl peroxide (6 g. mole of monomer) and 274 g. isopropanol. The bottle is rotated for 39 hrs. in a 50° C. bath and solids analysis indicates 88% conversion. The reaction product is neutralized with KOH and stripped. A 10% solution has a surface tension of 27.0 d./cm.

Run 5—n-Octyl-S-[acrylonitrile]-16-[acrylic acid]<sub>24</sub>-H

In a laboratory reactor are placed 21.2 g. acrylonitrile (0.4 moles), 43.2 g. acrylic acid (0.6 moles), 3.65 g. n-octyl mercaptan (0.025 moles) and 195 g. isopropanol. The reaction mix is heated to 70° C. and 1 g. lauroyl peroxide is added. The temperature rises to 73.4° C. Lauroyl peroxide is added: 1 g. at the end of 43 min. and 1 g. at the end of 103 min. from initial addition of lauroyl peroxide. Reaction is stopped at 6 hours. The conversion is 83.5%.

Run 6—n-Dodecyl-S-[acrylic acid]<sub>10</sub>-H

In a laboratory reactor are placed 72 g. acrylic acid (1 mole), 20.2 g. n-dodecyl mercaptan (0.1 mole), 1.5 g. lauroyl peroxide, and 275 g. isopropanol. The reaction is heated to 39.3° C. and 7 drops DMA (N,N-dimethyl

aniline) are added. The temperature rises to 46.7° C. in 1 hour. At 75 min., when temperature drops to 43.9° C., 8 drops DMA are added, which causes the temperature to rise to 45.4° C. Subsequent additions of 0.5 g. lauroyl peroxide and 5 drops DMA cause no exotherm. The reaction is stopped after 7.5 hours and the conversion is 98%. The reaction product is diluted with water and stripped free of alcohol.

Run 7—n-Dodecyl-S-[acrylic acid]<sub>20</sub>-H

This oligomer is prepared as in Run 6, except for use of 10.1 g. n-dodecyl mercaptan (0.05 moles). The reaction product is diluted with water and stripped free of methanol without neutralization.

Run 8—n-Dodecyl-S-[acrylonitrile]<sub>10</sub>-[acrylic acid]<sub>10</sub>-H

This oligomer is prepared as in Run 4 except for the use of 10.1 g. n-dodecyl mercaptan in place of the octyl mercaptan. 82% conversion is attained. The reaction mix is neutralized with aqueous KOH and stripped.

Run 9—n-Octyl-S-[methyl acrylate]<sub>5</sub>-[acrylic acid]<sub>15</sub>-H

In a laboratory reactor are placed 54 g. acrylic acid (0.75 moles), 21.5 g. methyl acrylate (0.25 moles) 7.3 g. n-octyl mercaptan (0.05 moles), 1.5 g. lauroyl peroxide, and 275 g. isopropanol. The reaction mix is heated to 39.3° C. with a water bath and 8 drops of DMA are added. The temperature rises to 47.0° C. in 40 min. and falls to 45.2° C. in the following 5 min. Thereafter 8 drops DMA are added and the temperature rises to 47.0° C. and then falls again to 40° C. in the following 90 min. The addition of 0.5 g. lauroyl peroxide and 5 drops DMA shows no exotherm. Conversion was 98.7%.

The reaction mix is diluted with water and stripped free of isopropanol. It is insoluble in water on standing and required KOH neutralization to become a homogeneous solution.

Run 10—n-Dodecyl-S-[methyl acrylate]<sub>5</sub>-[acrylic acid]<sub>15</sub>-H

This oligomer is prepared exactly as in Run 9 except for use of 10.1 g. dodecyl mercaptan (0.05 moles) in place of n-octyl mercaptan. Conversion is 99.5%. The reaction product is diluted with water and stripped free of isopropanol and is neutralized with KOH.

Run 11—R-S-[acrylic acid]<sub>5</sub>-[vinyl pyrrolidone]<sub>15</sub>-H

This oligomer is prepared in bottle reactors with 83.25 g. vinyl pyrrolidone, 18 g. acrylic acid and 0.05 moles of n-octyl mercaptan (7.3 g.), 6 g. lauroyl peroxide and 269 g. methanol. The reaction is conducted at 50° C. for 64 hours and a one phase reaction product results. The reaction if repeated with n-dodecyl mercaptan (10.1 g.). Solids indicate 88% conversion for the n-octyl type and 80% for the n-dodecyl.

Run 12—R-S-[acrylic acid]<sub>8</sub>-[vinyl pyrrolidone]<sub>12</sub>-H

This oligomer is prepared as in the previous run, except the reaction is run only 16 hours. Two phases formed in the bottle and solids indicate conversions of about 80%.

### EXAMPLE III

Data are presented, in Table 3, on the preparation and properties of materials represented by the formula, R-S-[A]<sub>a</sub>-[acrylamide]<sub>d</sub>-H, and in Table 4 similar information on R-S-[A]<sub>a</sub>-[methacrylamide]<sub>b</sub>-H, with [A] representing in both cases a polymerizable carboxylic acid.

The preparation of n-octyl-S-[itaconic acid]<sub>2</sub>-[acrylamide]<sub>18</sub>-H, is given in detail here. This general procedure is used for the other synthesis described in Tables 3 and 4.

A wide-mouth gallon jar is charged with 474.4 g. acrylamide, 96.5 g. itaconic acid, 54.2 g. n-octyl mercaptan, 18.6 g. lauroyl peroxide, and 2339 ml. isopropanol. The lid of the jar is fitted with an agitator, gas inlet and out-

let tube through which nitrogen flowed, and a liquid phase thermometer. This ensemble is placed in a 40° C. constant temperature bath. After 45 minutes the reaction mixture is homogeneous and at a temperature of 37.5° C. The subsequent performance is shown in Table 2.

TABLE 2  
[Oligomerization observations]

| Time in minutes | Temperature, °C. | N,N-di-methyl aniline added, ml. | Appearance         |
|-----------------|------------------|----------------------------------|--------------------|
| 0               | 37.5             | 2.7                              | Slight haze.       |
| 25              | 44.0             | 1.7                              | White precipitate. |
| 44              | 50.0             | —                                | —                  |
| 60              | 50.0             | —                                | —                  |
| 75              | 49.0             | 1.5                              | —                  |
| 95              | 45.0             | —                                | —                  |
| 135             | 40.0             | —                                | —                  |
| 162             | 39.0             | —                                | —                  |
| 175             | 39.0             | —                                | —                  |

The reaction mixture is vacuum filtered, and the retained precipitate is washed with 2500 ml. of isopropanol at room temperature and dried to content weight by drawing air through it. On drying this material at 105° C. in a vacuum oven, a weight loss of 5.6% occurred. The weight of white free-flowing powder is 580 g. or a 93% yield based on the weight of acrylamide, itaconic acid, and n-octyl mercaptan.

Analysis of this product shows 1.51% sulfur or 6.89% n-octyl mercaptan, 17.16% itaconic acid, and 14.70% nitrogen or 74.55% acrylamide and thus is essentially pure.

To show distribution of molecular size in this product, 54 g. is dissolved in 240 g. water to form a clear solution. 300 ml. isopropanol is added slowly with agitation. This forms a cloudy, but apparently homogeneous system, but on standing overnight separates into two clear layers. The upper layer is much larger. Separation of these layers and evaporation of solvent gives the following results:

| Material    | Weight, g. | Percent |               |
|-------------|------------|---------|---------------|
|             |            | Sulfur  | Itaconic acid |
| Original    | 54         | 1.51    | 17.16         |
| Upper layer | 40         | 1.82    | 16.68         |
| Lower layer | 13         | 0.63    | 17.02         |

These data show a non-uniform distribution of the sulfur. It is assumed here that the mercaptan determines the molecular size and that there is one sulfur per molecule. A fractionation would separate molecules according to size, so that it is expected that less sulfur would be present in the high molecular weight fraction. Distribution of itaconic acid is uniform however.

From the charge, the molecular weight of the product is calculated as 1684. Assuming one sulfur per molecule, 10 sulfur analysis shows a molecular weight of 2120, which would be expected since low molecular weight species are probably more soluble in isopropanol, and so do not appear in the product or are removed by washing. The freezing point depression of an aqueous solution of the product (5 g. in 95 g. water) is  $\Delta 0.105^\circ\text{C}$ . If the molar freezing point depression of the water for this polyelectrolyte were the same as 0.02 molar oxalic acid ( $\Delta 3.40^\circ\text{C}$ .) a molecular weight of 1704 would be indicated.

The product dissolved readily in water to make a 10% solution which had a viscosity of 2.1 centipoises at room temperature. The surface tension at various concentrations is given in the following tabulation:

| Concentration, percent: | Surface tension, d./cm. |
|-------------------------|-------------------------|
| 10                      | 44                      |
| 1                       | 40                      |
| 0.1                     | 51                      |
| 0.01                    | 60                      |
| 0.001                   | 69                      |

This is typical behavior of a surface active agent.

To show the solubility and surface activity of divalent salts of acidic polyamide sulfides, 1.05 g.  $\text{Ca}(\text{OH})_2$  is added to a 10% solution of this product containing 21.4 g. The amount of calcium hydroxide would neutralize half of the itaconic acid present. The resulting solution is 40 clear, had 2.3 cp. viscosity and shows a surface tension of 45 d./cm.

Following substantially the same procedure salts of monovalent cations, viz, sodium, potassium and ammonium, and other divalent cations, viz calcium, magnesium, zinc and barium, were prepared. All these salts dissolve in water sufficiently to form a 10% solution of low viscosity and surface tension.

Additional runs are summarized on Tables 3 and 4:

TABLE 3, PART I  
[Preparation and properties of  $\text{R-S-[A]}_n\text{-[acrylamide]}_b\text{-H}$  oligomers]

| Number                             | 2             | 3    | 4     | 5    | 6    | 7    | 8    | 9    | 10   | 11    | 12   | 13   | 14   | 15   | 16   | 17        |
|------------------------------------|---------------|------|-------|------|------|------|------|------|------|-------|------|------|------|------|------|-----------|
| Composition:                       |               |      |       |      |      |      |      |      |      |       |      |      |      |      |      |           |
| R                                  | n-Octyl       |      |       |      |      |      |      |      |      |       |      |      |      |      |      | n-Dodecyl |
| A                                  | Itaconic acid |      |       |      |      |      |      |      |      |       |      |      |      |      |      |           |
| $a+b$                              | 10            | 20   | 20    | 20   | 20   | 40   | 10   | 20   | 20   | 10    | 15   | 20   | 20   | 40   | 40   | 40        |
| $a/(a+b)$                          | 0.075         | 0.05 | 0.10  | 0.15 | 0.20 | 0.10 | 0.15 | 0.1  | 0.2  | 0.075 | 0.10 | 0.05 | 0.10 | 0.05 | 0.1  | 0.25      |
| Reaction:                          |               |      |       |      |      |      |      |      |      |       |      |      |      |      |      |           |
| Initial initiator <sup>d</sup>     | 1.2           | 1.7  | 2.5   | 1.4  | 1.5  | 1.5  | 0.4  | 0.75 | 0.3  | 1.5   | 2.3  | 2.1  | 1.82 | 1.4  | 1.5  | 1.3       |
| Incremental initiator <sup>d</sup> | 0             | 0    | 0     | 0.7  | 2.2  | 0    | 0.4  | 0    | 0    | 1.5   | 0    | 0    | 0    | 0.9  | 0.72 | 2.6       |
| Initial activator <sup>e</sup>     | 0.37          | 0.51 | 0.35  | 0.4  | 0.5  | 0.24 | 0.13 | 0.23 | 0.09 | 0.45  | 0.68 | 0.62 | 0.55 | 0.40 | 0.50 | 0.38      |
| Incremental activator <sup>e</sup> | 0             | 0    | 0.41  | 1.2  | 0.75 | 0.24 | 0.13 | 0    | 0.05 | 0.15  | 0.34 | 0    | 0    | 0.46 | 0.24 | 0.95      |
| Isopropanol <sup>f</sup>           | 350           | 350  | 350   | 350  | 438  | 350  | 500  | 450  | 400  | 400   | 350  | 350  | 350  | 476  | 350  | 400       |
| Time, min.                         | 150           | 190  | 175   | 170  | 200  | 285  | 160  | 135  | 355  | 165   | 155  | 145  | 175  | 128  | 270  | 150       |
| Yield, percent                     | 88            | 98   | 88    | 81   | 83   | 97   | 74   | 88   | 81   | 88    | 98   | 97   | 92   | 94   | 97   | 71        |
| Product analysis, percent:         |               |      |       |      |      |      |      |      |      |       |      |      |      |      |      |           |
| R-SH                               | 13.3          | 6.9  | 7.4   |      |      |      | 13.3 |      | 7.6  | 15.8  |      |      |      |      |      | 1.3       |
| Acrylamide                         | 75.9          | 74.5 | 68.9  |      |      |      | 75.2 |      | 74.0 | 72.2  |      |      |      |      |      | 55.8      |
| A                                  | 12.2          | 17.2 | 24.6  |      |      |      | 10.5 |      | 16.8 | 11.3  |      |      |      |      |      | 15.3      |
| Total                              | 101.4         | 98.6 | 100.9 |      |      |      | 99.0 |      | 98.4 | 99.3  |      |      |      |      |      | 98.0      |
| 10% aqueous solution:              |               |      |       |      |      |      |      |      |      |       |      |      |      |      |      |           |
| Viscosity, cp.                     | 1.8           | 2.1  |       | 3.0  |      | 2.1  |      |      | 2.2  |       | 3.1  |      |      |      |      |           |
| Surface tension, d./cm.            | 38            | 45   |       | 43   |      | 39   |      |      | 44   |       | 37   |      |      |      |      |           |

See footnotes at end of Table 3, Part II.

TABLE 3, PART II

[Preparation and properties of R-S-[A]<sub>a</sub>-[acrylamide]<sub>b</sub>-H oligomers]

| Number                             | 18           | 19    | 20   | 21    | 22   | 23          | 24   | 25   | 26   | 27   |
|------------------------------------|--------------|-------|------|-------|------|-------------|------|------|------|------|
| Composition:                       |              |       |      |       |      |             |      |      |      |      |
| R                                  | n-Dodecyl    |       |      |       |      | n-Octyl     |      |      |      |      |
| A                                  | Acrylic acid |       |      |       |      | Methacrylic |      |      |      |      |
| <i>a</i>                           | 20           | 40    | 40   | 15    | 15   | 20          | 20   | 20   | 20   | 20   |
| <i>a</i> + <i>b</i>                | 0.20         | 0.05  | 0.15 | 0.075 | 0.15 | 0.10        | 0.20 | 0.10 | 0.20 | 0.25 |
| <i>a</i> / <i>a</i> + <i>b</i>     |              |       |      |       |      |             |      |      |      |      |
| Reaction:                          |              |       |      |       |      |             |      |      |      |      |
| Initial initiator <sup>d</sup>     | 0.75         | 1.2   | 1.2  | 1.39  | 1.32 | 0.6         | 1.5  | 1.5  | 0.75 | 0.75 |
| Incremental initiator <sup>d</sup> | 0.55         | 0     | 0    | 0     | 2.64 | 1.2         | 1.5  | 0    | 0.38 | 0.38 |
| Initial activator <sup>e</sup>     | 0.12         | 0.3   | 0.3  | 0.41  | 0.40 | 0.21        | 0.44 | 0.51 | 0.12 | 0.12 |
| Incremental activator <sup>e</sup> | 0.28         | 0     | 0    | 0     | 1.00 | 0.53        | 0.88 | 0    | 0.25 | 0.25 |
| Isopropanol <sup>f</sup>           | 450          | 516   | 576  | 538   | 493  | 450         | 450  | 349  | 450  | 450  |
| Time, min.                         | 255          | 119   | 114  | 155   | 183  | 215         | 180  | 75   | 190  | 210  |
| Yield, percent                     | 84           | 92    | 94   | 69    | 82   | 87          | 94   | 85   | 89   | 89   |
| Product analysis, percent:         |              |       |      |       |      |             |      |      |      |      |
| RSH                                |              | 1.8   | 4.2  |       |      |             | 6.6  |      |      |      |
| Acrylamide                         |              | 84.8  | 77.6 |       |      |             | 63.8 |      |      |      |
| A                                  |              | 15.3  | 16.6 | 5.6   | 6.0  |             | 20.3 | 5.8  |      |      |
| Total                              |              | 101.9 | 98.4 |       |      |             | 96.7 |      |      |      |
| 10% aqueous solution:              |              |       |      |       |      |             |      |      |      |      |
| Viscosity, cp                      | 3.0          |       |      | 1.0   | 2.2  |             |      | 2.5  | 2.4  |      |
| Surface tension, d./cm             | 46           |       |      | 44    | 35   |             |      | 50   | 47   |      |

<sup>d</sup> Initiator, lauroyl peroxide as g./mole of monomers.<sup>e</sup> Activator, N,N-dimethyl aniline as g./mole of monomers.<sup>f</sup> Isopropanol: ml./mole acrylamide.<sup>g</sup> The R was n-octyl/n-dodecyl in mole ratio of 9/1.<sup>h</sup> The R was n-octyl/n-dodecyl in mole ratio of 975/25.

## EXAMPLE IV

TABLE 4  
[Preparation and properties of R-S-[A]<sub>a</sub>-[methacrylamide]<sub>b</sub>-H oligomers]

| Number                                   | 28                               | 29                               | 30                                | 30 |
|------------------------------------------|----------------------------------|----------------------------------|-----------------------------------|----|
| R                                        | n-C <sub>8</sub> H <sub>17</sub> | n-C <sub>8</sub> H <sub>17</sub> | n-C <sub>12</sub> H <sub>25</sub> |    |
| A                                        | (1)                              | (3)                              | (2)                               |    |
| <i>a</i> + <i>b</i>                      | 20                               | 20                               | 20                                |    |
| <i>a</i> / <i>a</i> + <i>b</i>           | 0.2                              | 0.1                              | 0.1                               |    |
| Lauroyl peroxide, g./mole, monomers:     |                                  |                                  |                                   |    |
| Initial                                  | 2.5                              | 2.5                              | 2.5                               | 35 |
| Incremental                              | 2.5                              |                                  |                                   |    |
| N,N-dimethyl aniline, g./mole, monomers: |                                  |                                  |                                   |    |
| Initial                                  | 0.75                             |                                  |                                   |    |
| Incremental                              | 1.87                             |                                  |                                   |    |
| Isopropanol, g./mole methacrylamide      | 500                              | 274                              | 274                               |    |
| Reaction time, hr                        | 4 160                            | 64                               | 64                                | 40 |
| Yield, percent                           | 83                               | 63                               | 73                                |    |
| Product analysis, percent:               |                                  |                                  |                                   |    |
| RSH                                      | 1.6                              |                                  |                                   |    |
| Methacrylamide                           | 81.7                             |                                  |                                   |    |
| Acid                                     | 13.5                             |                                  |                                   |    |
| Total                                    | 96.8                             |                                  |                                   |    |
| 10% aqueous solution viscosity, cp       |                                  |                                  |                                   |    |
|                                          | 2.8                              |                                  |                                   |    |

<sup>1</sup> Acrylic acid.<sup>2</sup> Itaconic acid.<sup>3</sup> These runs are made in bottle reactors at 50° C.<sup>4</sup> Minutes.The data of this example show, in Table 5, the preparation and properties of materials represented by the formula: R-S-[acrylamide]<sub>a</sub>-H.The preparation of n-dodecyl-S-[acrylamide]<sub>15</sub>-H is given in detail, this procedure being used for all syntheses described in Table 5.

The jar reactor is loaded with 80.2 g. acrylamide, 1.4 g. lauroyl peroxide, 565 ml. isopropanol, and 15.2 g. primary dodecyl mercaptan. Nitrogen is passed through the vapor phase of the reactor while the contents are agitated. The reactor is in a 40° C. thermostated bath. After 25 minutes 0.39 g. N,N-dimethyl aniline (DMA) is added through the reflux condenser. Three minutes thereafter the reaction materials turn cloudy and their temperature increases, reaching 45° C. in 18 minutes and then falling to the bath temperature in 103 minutes after the addition of the DMA. The reaction mixture is filtered immediately using a vacuum system. The precipitate is washed with 500 ml. of isopropanol and dried by drawing an air stream through it overnight.

The free-flowing white precipitate is then dried for 3 hours in a vacuum oven at 110–112° C. The weight of 50 the product indicates a yield of 83% based on the amount of acrylamide plus mercaptan.

TABLE 5  
[Preparation and properties of R-S-[acrylamide]<sub>a</sub>-H oligomers]

| Number                                   | 1                                | 2                                 | 3                                 | 4                                 | 5                                 | 6                                 |
|------------------------------------------|----------------------------------|-----------------------------------|-----------------------------------|-----------------------------------|-----------------------------------|-----------------------------------|
| Composition:                             |                                  |                                   |                                   |                                   |                                   |                                   |
| R                                        | n-C <sub>8</sub> H <sub>13</sub> | n-C <sub>10</sub> H <sub>21</sub> | n-C <sub>10</sub> H <sub>21</sub> | n-C <sub>12</sub> H <sub>25</sub> | n-C <sub>12</sub> H <sub>25</sub> | n-C <sub>10</sub> H <sub>23</sub> |
| <i>a</i>                                 | 15                               | 15                                | 40                                | 5                                 | 15                                | 15                                |
| Reaction conditions, 40° C.:             |                                  |                                   |                                   |                                   |                                   |                                   |
| Lauroyl peroxide, g./mole, monomers:     |                                  |                                   |                                   |                                   |                                   |                                   |
| Initial                                  | 0.7                              | 0.7                               | 1.2                               | 1.2                               | 1.2                               | 0.7                               |
| Incremental                              | 1.0                              | 0                                 | 0                                 | 0                                 | 0                                 | 1.0                               |
| N,N-dimethyl aniline, g./mole, monomers: |                                  |                                   |                                   |                                   |                                   |                                   |
| Initial                                  | 0.2                              | 0.15                              | 0.3                               | 0.33                              | 0.35                              | 0.19                              |
| Incremental                              | 0                                | 0                                 | 0                                 | 0                                 | 0                                 | 0                                 |
| Isopropanol, g./mole acrylamide          | 300                              | 300                               | 490                               | 500                               | 500                               | 300                               |
| Reaction time, minutes                   | 82                               | 76                                | 100                               | 81                                | 103                               | 72                                |
| Yield, percent                           | 94                               | 90                                | 88                                | 34                                | 83                                | 96                                |
| Product analysis, percent:               |                                  |                                   |                                   |                                   |                                   |                                   |
| RSH                                      |                                  |                                   |                                   | 26.4                              | 14.3                              |                                   |
| Acrylamide                               |                                  |                                   |                                   | 73.5                              | 85.7                              |                                   |
| Total                                    |                                  |                                   |                                   | 99.9                              | 100.0                             |                                   |
| 10% aqueous solution:                    |                                  |                                   |                                   |                                   |                                   |                                   |
| Viscosity, cp                            |                                  |                                   |                                   | 3.4                               | 1.7                               | 2.7                               |
| Surface tension, d./cm                   |                                  |                                   |                                   | 49                                | 40                                | 46                                |

15  
EXAMPLE V

This example demonstrates the preparation and properties of N-dodecyl-S-[methacrylamide]<sub>15</sub>-H.

In a bottle reactor is placed 42.5 g. methacrylamide, 1.2 g. lauryl peroxide, 0.3 g. N,N-dimethyl aniline, 250 ml. isopropanol and 6.73 g. primary dodecyl mercaptan. The bottle is flushed with nitrogen, capped, and rotates overnight in a 50° C. bath. The bottle is cooled, opened and the contents are filtered. The precipitate is washed with 250 ml. of isopropanol and then dried first in an air stream and then in a vacuum oven for 3 hours. A yield of 70% is obtained. A 10% aqueous solution of this material has a surface tension of 41.8 d./cm. and a viscosity of 3.0 centipoises. Analysis of the product shows 10.3% n-dodecyl mercaptan and 86.8% acrylamide.

## EXAMPLE VI

The preparation and properties of n-dodecyl-S-[ethylacrylate]<sub>a</sub>-[acrylamide]<sub>b</sub>-H type materials are presented here.

$$\text{Run 1: } \frac{a}{a+b} = 0.05; a+b=40$$

A reactor is run for 75 minutes at 40° C. containing 33.7 g. acrylamide, 2.5 g. ethyl acrylate, 2.53 g. normal dodecyl mercaptan, 1 g. lauryl peroxide, 0.25 g. N,N-dimethyl aniline, and 250 ml. ethanol. The dry precipitate from this reaction indicates 95% yield and as a 10% aqueous solution shows 40.5 d./cm. surface tension and 6.0 centipoises viscosity.

$$\text{Run 2: } \frac{a}{a+b} = 0.15; a+b=40$$

A reactor is run for 75 minutes at 40° C. containing 30.2 g. acrylamide, 7.51 g. ethyl acrylate, 2.53 g. n-dodecyl mercaptan, 1 g. lauryl peroxide, 0.25 g. N,N-dimethyl aniline and 250 ml. ethanol. The dried precipitate indicates 95% conversion.

## EXAMPLE VII

This example demonstrates the preparation and properties of n-dodecyl-S-[vinyl pyrrolidone]<sub>4</sub>-[acrylamide]<sub>36</sub>-H.

A jar reactor is run for 75 minutes at 40° C. containing 32 g. acrylamide, 5.55 g. vinyl pyrrolidone, 2.53 g. normal dodecyl mercaptan, 1 g. lauryl peroxide, 0.25 g. N,N-dimethyl aniline and 250 ml. ethanol. The yield is 94%. The product, as a 10% aqueous solution, shows 37.2 d./cm. surface tension and 5.8 centipoises viscosity.

## EXAMPLE VIII

The preparation of n-octyl-S-[N-isopropyl acrylamide]<sub>4</sub>-[acrylamide]<sub>16</sub>-H is described here. The following ingredients are stirred under nitrogen for 65 minutes at 40° C.; 54 g. acrylamide, 21.5 g. N-isopropyl acrylamide, 6.94 g. n-octyl mercaptan, 2.3 g. lauryl peroxide, 0.64 g. N,N-dimethyl aniline and 421 ml. isopropanol. This reaction mixture does not pass through filter paper readily and the product is isolated by evaporation of the isopropanol. The tan powder resulting is soluble in water.

## EXAMPLE IX

The preparation and properties of n-octyl-S-[vinyl ethyl ether]<sub>2</sub>-[acrylamide]<sub>18</sub>-H are shown in this example.

A bottle reactor containing 66.4 g. acrylamide, 7.49 g. vinyl ethyl ether, 7.58 g. n-octyl mercaptan, 1.0 g. lauryl peroxide, and 421 ml. isopropanol was agitated at 50° C. for 16 hours. The precipitate which forms is collected by filtration, washed with 421 ml. isopropanol, and dried. The yield is 85%.

A 10% aqueous solution of this powder has 46 d./cm. surface tension and 2.0 centipoise viscosity.

16  
EXAMPLE X

This example describes the preparation of n-dodecyl-S-[hydroxyethyl methacrylate]<sub>a</sub>-[acrylamide]<sub>b</sub>-H.

A reactor containing 39.05 g. acrylamide, 12.6 g. hydroxyethyl methacrylate, 3.27 g. n-dodecyl mercaptan, 0.8 g. lauryl peroxide, and 500 ml. isopropanol, is heated in a 40° C. water bath and 0.028 g. N,N-dimethyl aniline added. The reaction is run 205 minutes and during this time, 1 g. lauryl peroxide and 0.7 g. N,N-dimethyl aniline is added. The dried precipitate from this reaction is soluble in water. The yield is 99%.

## EXAMPLE XI

In this example, the preparation of n-dodecyl-S-[vinyl acetate]<sub>a</sub>-[acrylamide]<sub>b</sub>-H type materials is described.

$$\text{Run 1: } \frac{a}{a+b} = 0.2; a+b=40$$

In a reactor are placed 58.4 g. acrylamide, 17.7 g. vinyl acetate, 5.2 g. n-dodecyl mercaptan, 1.2 g. lauryl peroxide, and 500 ml. isopropanol. The contents are heated to 40° C. and 0.34 g. N,N-dimethyl aniline (DMA) added. At 25 minutes 0.17 g. DMA is added. After 65 minutes the reaction mixture is filtered and the retained precipitate washed with 500 ml. isopropanol before drying. The yield is 75%.

$$\text{Run 2: } \frac{a}{a+b} = 0.4; a+b=40$$

This differed from Run 1 in the amount of acrylamide (43.8 g.), amount of vinyl acetate (35.4 g.), amount of incremental DMA (0.7 g.), use of 2.4 g. incremental lauryl peroxide and reaction time of 135 minutes. The yield is 72%.

## EXAMPLE XII

The preparation and properties of n-dodecyl-S-[acrylonitrile]<sub>a</sub>-[acrylamide]<sub>b</sub>-H is described in this example.

Heated to 40° are 57.4 g. acrylamide, 10.7 g. acrylonitrile, 5.1 g. n-dodecyl mercaptan, 1.2 g. lauryl peroxide, and 500 ml. isopropanol. Then, 0.34 g. N,N-dimethyl aniline are added. The reaction is run 165 minutes and during this time 1.2 g. lauryl peroxide and 0.68 g. DMA are added. The dried product represents 79% yield and, as a 10% aqueous solution, has 3 centipoises viscosity and 38 d./cm. surface tension.

## EXAMPLE XIII

Materials of the n-dodecyl-S-[methyloacrylamide]<sub>a</sub>-[acrylamide]<sub>b</sub>-H type are described in this example.

$$\text{Run 1: } \frac{a}{a+b} = 0.167; a+b=15$$

A reactor containing 71 g. acrylamide, 20.2 g. methyloacrylamide, 16.2 g. n-dodecyl mercaptan, 1.2 g. lauryl peroxide, 0.3 g. N,N-dimethyl aniline and 470 ml. isopropanol is held at 40° C. for 70 minutes. The product is removed by filtration and, when dry, indicates 90% yield. The product is not completely soluble in water as a 10% solution.

$$\text{Run 2: } \frac{a}{a+b} = 0.15; a+b=39$$

In a reactor are placed 71 g. acrylamide, 18.1 g. methyloacrylamide, 6.1 g. n-dodecyl mercaptan, 1.2 g. lauryl peroxide, 0.3 g. N,N-dimethyl aniline and 485 ml. isopropanol. The reaction mixture is heated to 40° C. and maintained at that temperature for 60 minutes. The dried precipitate, which indicates an 87% yield, is dissolved in water to make a 10% solution.

## EXAMPLE XIV

The data of this example show, in Table 6, the preparation and properties of materials represented by the formula R-S-[glycidyl methacrylate]<sub>a</sub>-[acrylamide]<sub>b</sub>-H.

The syntheses and behavior of a specific product are given in detail.

Run 1: n-Dodecyl-S-[glycidyl methacrylate]<sub>3</sub>-[acrylamide]<sub>12</sub>-H

A reaction vessel in a 38.2° C. thermostatted bath, there is agitated, under nitrogen, 71 g. acrylamide, 35.5 g. glycidyl methacrylate, 16.8 g. normal dodecyl mercaptan, 3 g. lauroyl peroxide, 0.75 g. N,N-dimethyl aniline and 463 ml. isopropanol. The reaction temperature rises to 40.9° C. after 107 minutes and then starts to fall. Thereafter, 1 g. lauroyl peroxide and 0.25 g. N,N-dimethyl aniline are added, but the temperature continues to fall. At 225 minutes, the mixture is filtered and the collected precipitate dried in an air stream. This is a white free-flowing powder. The yield is 81% based on weight of acrylamide, glycidyl methacrylate and n-dodecyl mercaptan. Analysis of this product showed 10.4% n-dodecyl mercaptan, 60.9% acrylamide, and 27.4% glycidyl methacrylate for a total of 98.7%.

This product dissolves in water to make a 10% solution having a viscosity of 4 centipoises. On standing overnight at room temperature a precipitate forms. When the fresh solution is evaporated on a steam cone, the solid does not dissolve in, but is swollen by water. Thus this polyepoxide is apparently self cross-linking.

Table 6 summarizes the above and other runs:

TABLE 6

| Number                                         | [Preparation and properties of R-S-[glycidyl methacrylate] <sub>a</sub> -[acrylamide] <sub>b</sub> -H oligomers] | 1                                | 2                                 | 3                                 | 4                                 | 5                                 | 6 |
|------------------------------------------------|------------------------------------------------------------------------------------------------------------------|----------------------------------|-----------------------------------|-----------------------------------|-----------------------------------|-----------------------------------|---|
| Composition:                                   |                                                                                                                  |                                  |                                   |                                   |                                   |                                   |   |
| R                                              | n-C <sub>12</sub> H <sub>25</sub>                                                                                | n-C <sub>8</sub> H <sub>17</sub> | n-C <sub>12</sub> H <sub>25</sub> | n-C <sub>12</sub> H <sub>25</sub> | n-C <sub>12</sub> H <sub>25</sub> | n-C <sub>12</sub> H <sub>25</sub> |   |
| a+b                                            | 15                                                                                                               | 40                               | 20                                | 20                                | 40                                | 40                                |   |
| a/(a+b)                                        | 0.20                                                                                                             | 0.20                             | 0.08                              | 0.17                              | 0.20                              | 0.20                              |   |
| Reaction conditions (O <sub>2</sub> , 40° C.): |                                                                                                                  |                                  |                                   |                                   |                                   |                                   |   |
| Lauroyl peroxide, g./mole, monomers:           |                                                                                                                  |                                  |                                   |                                   |                                   |                                   |   |
| Initial                                        | 2.4                                                                                                              | 1.26                             | 2.4                               | 2.0                               | 1.52                              | 2.2                               |   |
| Incremental                                    | 0.8                                                                                                              | 1.52                             | 0                                 | 0                                 | 1.52                              | 0.65                              |   |
| N,N-dimethyl aniline, g./mole, monomers:       |                                                                                                                  |                                  |                                   |                                   |                                   |                                   |   |
| Initial                                        | 0.6                                                                                                              | 0.35                             | 0.6                               | 0.5                               | 0.42                              | 0.61                              |   |
| Incremental                                    | 0.2                                                                                                              | 1.75                             | 0                                 | 0                                 | 1.26                              | 0.61                              |   |
| Isopropanol, ml./mole acrylamide               | 463                                                                                                              | 656                              | 470                               | 392                               | 631                               | 678                               |   |
| Time, minutes                                  | 225                                                                                                              | 115                              | 90                                | 169                               | 120                               | 135                               |   |
| Yield, percent                                 | 81                                                                                                               | 78                               | 75                                | 87                                | 91                                | 91                                |   |
| Product analysis, percent:                     |                                                                                                                  |                                  |                                   |                                   |                                   |                                   |   |
| RSH                                            | 10.4                                                                                                             |                                  |                                   |                                   | 1.7                               |                                   |   |
| Acrylamide                                     | 60.9                                                                                                             |                                  |                                   |                                   | 63.1                              |                                   |   |
| Glycidyl methacrylate                          | 27.4                                                                                                             | 18.9                             |                                   |                                   | 31.4                              |                                   |   |
| Total                                          | 98.7                                                                                                             |                                  |                                   |                                   | 96.2                              |                                   |   |
| Properties:                                    |                                                                                                                  |                                  |                                   |                                   |                                   |                                   |   |
| 1 g. product soluble in 9 g. H <sub>2</sub> O  | Yes                                                                                                              | Yes                              | Yes                               | Yes                               | Yes                               | Yes                               |   |
| Product insolubilized when dried at 100° C.    | Yes                                                                                                              | Yes                              | Yes                               | Yes                               | Yes                               | Yes                               |   |

## EXAMPLE XV

In this example, the preparation and properties of n-dodecyl-S-[glycidyl acrylate]<sub>6</sub>-[acrylamide]<sub>34</sub>-H are described.

44.2 g. acrylamide, 14.1 g. glycidyl acrylate, 3.7 g. n-dodecyl mercaptan, 1.2 g. lauroyl peroxide, 0.4 g. N,N-dimethyl aniline, and 370 ml. isopropanol are agitated under nitrogen in a vessel which is in a 40° C. bath. The temperature of the reaction rises to 44.9° C. after 20 minutes then falls despite additional lauroyl peroxide (1.2 g.) and N,N-dimethyl aniline (0.8 g.). After 67 minutes the product is removed by filtration and dried in an air stream. The yield is 95% based on monomers and mercaptan. The product shows 20.6% glycidyl acrylate.

The free-flowing white powder dissolved in water to make a 10% solution. The product became insoluble after heating the solution to dryness on a steam bath.

Having thus described my invention, what I claim and desire to protect by Letters Patent is:

## 1. An oligomer having the formula:



wherein R is a straight or branched chain primary, sec-

75 is 0.05.

ondary or tertiary alkyl group having from 5 to 20 carbon atoms; R<sub>1</sub> and R<sub>3</sub> are hydrogen, methyl, ethyl or —COOH; R<sub>2</sub> and R<sub>4</sub> are hydrogen, methyl, ethyl, —COOH or CH<sub>3</sub>COOH; Y is a strongly polar group selected from the group consisting of —COOH, —CONH<sub>2</sub>, —OCH<sub>3</sub>, —OC<sub>2</sub>H<sub>5</sub> and —CH<sub>2</sub>OH; X is a different polar group selected from the group consisting of the foregoing strongly polar groups and

5 —COOC<sub>2</sub>H<sub>4</sub>OH, —COOC<sub>3</sub>H<sub>6</sub>OH, —CONHCH<sub>2</sub>OH, —CONHCH<sub>3</sub>, —CONHC<sub>2</sub>H<sub>5</sub>, —CONHC<sub>3</sub>H<sub>7</sub>, —COOCH<sub>3</sub>, —COOC<sub>2</sub>H<sub>5</sub>, —CN, —OOCCH<sub>3</sub> and —OOCCH<sub>2</sub>H<sub>5</sub>; a+b is from 2 to 50; and

10  $\frac{a}{a+b}$

is from 0.05 to 0.6; and, where the oligomer has at least one carboxylic acid group, the said group may be in the form of the free acid or the alkaline salt thereof.

20 2. The oligomer of claim 1 wherein R is primary alkyl having 6 to 12 carbon atoms; R<sub>1</sub>, R<sub>2</sub>, R<sub>3</sub> and R<sub>4</sub> are hydrogen; X is a —CN group; Y is a —COOH group; a+b is from 4 to 50; and

25  $\frac{a}{a+b}$

is from 0.2 to 0.6.

|                                               |     |     |     |     |     |     |  |
|-----------------------------------------------|-----|-----|-----|-----|-----|-----|--|
| Properties:                                   |     |     |     |     |     |     |  |
| 1 g. product soluble in 9 g. H <sub>2</sub> O | Yes | Yes | Yes | Yes | Yes | Yes |  |
| Product insolubilized when dried at 100° C.   | Yes | Yes | Yes | Yes | Yes | Yes |  |

3. The oligomer of claim 2 wherein R is a primary alkyl group with from 7 to 11 carbon atoms; a+b is from 12 to 30; and

35  $\frac{a}{a+b}$

is from 0.2 to 0.55.

4. The oligomer of claim 2 wherein R is straight chain primary octyl; a+b is 16; and

40  $\frac{a}{a+b}$

is 0.5.

5. The oligomer of claim 2 wherein R is straight chain primary decyl; a+b is 16; and

45  $\frac{a}{a+b}$

is 0.05.

6. The oligomer of claim 2 wherein R is primary dodecyl; a+b is 16; and

50  $\frac{a}{a+b}$

7. The oligomer of claim 1 wherein R is a primary alkyl group having from 7 to 12 carbon atoms; R<sub>1</sub>, R<sub>3</sub> and R<sub>4</sub> are hydrogen; R<sub>2</sub> is hydrogen or —CH<sub>2</sub>COOH; X is —COOH; Y is —CONH<sub>2</sub>; a+b is from 6 to 50; and

$$\frac{a}{a+b}$$

is 0.075 to 0.2.

8. The oligomer of claim 7 wherein R is a primary alkyl group having from 8 to 10 carbon atoms; R<sub>2</sub> is —CH<sub>2</sub>COOH; a+b is from 12 to 30; and

$$\frac{a}{a+b}$$

is from 0.075 to 0.15.

9. The oligomer of claim 7 wherein R is n-octyl; R<sub>2</sub> is —CH<sub>2</sub>COOH; a+b is 20; and

$$\frac{a}{a+b}$$

is 0.1.

10. The oligomer of claim 7 wherein R is primary octyl; R<sub>2</sub> is hydrogen; a+b is 20; and

$$\frac{a}{a+b}$$

5 is 0.20.

No references cited.

DONALD G. DAUS, Primary Examiner

J. TOVAR, Assistant Examiner

U.S. Cl. X.R.

15 260—29.6, 29.7, 78.5, 80.7, 80.8, 80.81, 82.1, 82.7, 84.3,  
85.5, 85.7, 86.1, 86.7, 88.1, 88.7, 89.5, 93.5, 326.22,  
326.45, 348 A, 34 R, 429.1, 429.2, 429.9, 465.5 R,  
465.6, 481 R, 501.1, 501.11, 501.12, 501.17, 501.21, 543  
B, 535 R, 537 S, 540, 541, 561 S, 614, 615 R, 615 P,  
632, 635 R

20

UNITED STATES PATENT OFFICE Page 1 of 2  
CERTIFICATE OF CORRECTIONPatent No. 3,839,405Dated October 1, 1974Inventor(s) Leland E. Dannals

It is certified that error appears in the above-identified patent and that said Letters Patent are hereby corrected as shown below:

Column 2, line 6: " $\text{CH}_2\text{COOH}$ " should read  $--\text{CH}_2\text{COOH}--$ .

line 17 (first formula): " $-\text{COOCH}_2\text{H}_4\text{OH}$ " should read

$--\text{COOC}_2\text{H}_4\text{OH}--$ .

line 23 (second formula): " $-\text{OOCH}_2\text{H}_5$ " should read

$--\text{OOCC}_2\text{H}_5--$ .

Column 4, line 5: " $\text{R-S-(CH}_2\text{-CR}_1\text{COOH})_a-\left(\text{CH}_2\text{-CR}_2\text{CONH}_2\right)_b\text{H}$ "

should read  $--\text{R-S-}\left(\text{CH}_2\text{-CR}_1\text{COOH}\right)_a-\left(\text{CH}_2\text{-CR}_2\text{CONH}_2\right)_b\text{H}--$ .

Column 5, Formula 17 (within the left pair of brackets):

"  $\text{CH}_2\text{-CH}$  " should read  $--\text{CH}_2\text{-CH}$  --.



Column 5, Formula 24 (within the left pair of brackets):

"  $\text{CH}_3$  " should read  $--\text{CH}_3$



Column 7, line 58: "additional" should read --addition--.

UNITED STATES PATENT OFFICE Page 2 of 2  
CERTIFICATE OF CORRECTION

Patent No. 3,839,405 Dated October 1, 1974  
Inventor(s) Leland E. Dannals

It is certified that error appears in the above-identified patent and that said Letters Patent are hereby corrected as shown below:

Column 8, line 3: "38" should read --39--;  
line 74: "mols" should read --moles--.

Column 9, line 59:  
"Run 5--n-Octyl-S-[acrylonitrile]-16-[acrylic acid]<sub>24-H</sub>"  
should read  
--Run 5--n-Octyl-S-[acrylonitrile]<sub>16-[acrylic acid]<sub>24-H</sub></sub>--.

Column 10, line 14 "methanol" should read --isopropanol--;  
line 52: "if" should read --is--;  
line 65: "R-S-[A]<sub>a</sub>-[acrylamide]<sub>d-H</sub>" should read  
-- R-S-[A]<sub>a</sub>-[acrylamide]<sub>b-H</sub>--.

Column 13, Table 4, in line "Yield, percent", in column "29":  
"63" should read --36--.

Column 15, line 3: "N-dodecyl" should read --n-dodecyl--;  
line 5: "lauryl" should read --lauroyl--.

Columns 17-18, Table 6, in line "R", in column "6":  
"n-C<sub>12</sub>H<sub>25</sub>" should read --n-C<sub>16</sub>H<sub>33</sub>--;

in line "Lauroyl peroxide, g./mole, monomers: Incremental", in column "6": "65" should read --1.65--.

Column 18, line 4: "CH<sub>2</sub>COOH" should read --CH<sub>2</sub>COOH--;  
line 69: "0.05" should read --0.5--.  
line 75: "0.05" should read --0.5--.

Signed and sealed this 13th day of May 1975.

(SEAL)  
Attest:

RUTH C. MASON  
Attesting Officer

C. MARSHALL DANN  
Commissioner of Patents  
and Trademarks